

# United States Patent Office

2,870,008

Patented Jan. 20, 1959

1

2,870,008

## ZINC-ALUMINIUM ALLOYS AND THE METHOD FOR PRODUCING SAME

Willi Neu, Saarbrücken, Saarland, assignor to Main Alloy Company Establishment (Mace), Vaduz, Liechtenstein

No Drawing. Application November 15, 1955  
Serial No. 547,045

Claims priority, application Great Britain  
November 18, 1954

5 Claims. (Cl. 75—141)

The present invention relates to zinc-aluminium alloys and the production thereof.

|         | Be                               | Al         | Zn        | Cu              | Si                   | Cr   | Ni             | Other metals | Uses                                                                                                                                 |
|---------|----------------------------------|------------|-----------|-----------------|----------------------|------|----------------|--------------|--------------------------------------------------------------------------------------------------------------------------------------|
| 1.....  | { 0.005<br>-0.01<br>-0.5         | 28.....    | Remainder | { 0.55<br>-1.26 | 1.10.....            |      |                | Mg 0.01..... | Casting and malleable alloys; corrosion-resistant bearings, cocks, possibly wires with subsequent treatment, good surface formation. |
| 2.....  | { 0.03<br>-0.35                  | 38.....    | do.....   | 2.00            | { 0.15<br>-1.20      |      | { 0.02<br>0.16 |              | Casting and malleable alloys, corrosion-resistant bearings resistant to sea water, plates, rapidly moving machine parts.             |
| 3.....  | 0.005                            | 28.....    | { do..... |                 | { 0.15               |      |                |              | Corrosion-resistant bearings, injection moulding, chill casting, cages for ball bearings.                                            |
| 4.....  | -0.455                           | 38.....    |           |                 | { 0.45               |      |                |              |                                                                                                                                      |
| 5.....  | 0.08                             | 36.....    | do.....   | 2.50            | { 0.15<br>1.50       |      | { 0.03<br>0.16 |              | Fine-grained, ductile, hard, pressable, bars, plates, bearings, wire, corrosion-resistant pump parts, rapidly moving machine parts.  |
| 6.....  | -1.50                            | 36.....    |           |                 |                      |      |                |              |                                                                                                                                      |
| 7.....  | 0.03                             | 32.....    | { do..... | { 2.00<br>3.20  | 0.15<br>1.50<br>3.20 | 0.03 |                |              | Casting and malleable alloys, corrosion-resistant bearing and machine parts resistant to sea water.                                  |
| 8.....  | -1.45                            | 32.....    |           |                 |                      |      |                |              |                                                                                                                                      |
| 9.....  | 0.60                             | 35.5.....  | do.....   | 2.20            | 1.35.....            |      | 0.12.....      |              | Bearings, corrosion-resistant pump parts, parts resistant to weak organic and weak inorganic acids and bases.                        |
| 10..... | 0.50                             | 35.5.....  | { do..... | 2.20            | { 1.35<br>2.25       |      | 0.12           | B 0.15.....  | Pressure-cast bearings, corrosion-resistant plates, electrical parts, wires.                                                         |
| 11..... | 0.50                             | 35.5.....  |           |                 |                      |      |                |              |                                                                                                                                      |
| 12..... | 0.50                             | 26.5.....  | do.....   | 0.55            | 0.45                 |      |                | MG traces.   | Concentrated alloys, bearings, key alloys for corrosion-resistant machine and pump parts.                                            |
| 13..... | 2.60                             | 50.00..... | do.....   | 4.55            | 2.50                 |      |                |              |                                                                                                                                      |
| 14..... | 4.5                              | 55.0.....  | do.....   | 8.00            | 6.5.....             |      | 0.12           | Ca 0.6.....  | Concentrated alloys for bearings, key alloys for machine and pump parts, corrosion-resistant and sea water resistant material.       |
| 15..... | { 0.08<br>-0.45<br>0.03<br>-0.35 | Remainder  | 28.....   | 3.8             | 0.33.....            |      |                |              | Bars, sleeves, wires, rollers, sheets.                                                                                               |
| 16..... |                                  | do.....    | 32.....   | 0.08            | 0.65.....            |      | 0.06.....      |              | Bars, sleeves, wire, bearings, pump parts.                                                                                           |

Alloys according to the present invention consist essentially of from 20% to 75% of aluminium, from 0.15% to 16% of silicon, from traces up to 10% of beryllium and zinc, the content of zinc being at least 20%. The term "consisting essentially of" used herein and in the claims hereof is intended to mean that the alloy may include one or more of the following optional elements, viz., calcium, sodium, strontium, barium, cadmium, tin, vanadium, molybdenum, manganese, cerium, potassium and/or incidental ingredients such as iron up to 3% which are used in known small quantities in connection with zinc-aluminium alloys, save that the sum of the said optional elements does not exceed 6%, and save that preferably

The zinc and aluminium may form the initial melt and the other elements be added thereto, either as free elements or as key alloys or chemical compounds. Certain of the elements and particularly the optional elements, notable calcium, sodium or strontium, may be added in the form of hydrides of the metals.

In preparing the melt, the silicon may be wholly or in part replaced by phosphorus or one or more other non-metals, e. g., carbon (preferably in the form of graphite).

The improved alloy has good acid-resisting and alkali resisting properties and is particularly suitable when a light-weight alloy is required which shall have these properties.

The alloy may be employed in the construction of pumps or parts of pumps, especially for pumping acids or alkalis, and for such and other purposes may replace steel, cast iron and bronzes with advantage. The alloy may be employed advantageously for bearings, bearing linings, and sliding, e. g., reciprocating, parts. It can be used as a key alloy or for workpieces, of various kinds and can be produced in sheet or wire form.

The melt may be cast by conventional methods in sand or chill moulds, or a bar or ingot may be partially chill-cast or semi-chill-cast, e. g., the molten alloy material may be caused to run down directly from a sand mould into a metal mould which is chilled so that a bar or ingot is formed which is contained partly in the metal mould and partly in the sand mould so as to cause a progressive chilling from the bottom of the bar or ingot to the top, or in other words, a quick solidification realised over the lower regions in particular of the bar or ingot.

Alloys according to the invention are amenable to pressure casting, centrifugal casting or vibration casting, e. g., the mould may be subjected to ultra-sonic oscillation. High compression characteristics can thereby be produced in the casting process.

The alloy may with advantage be used to replace screw-threaded parts of steel, cast iron or bronze.

The alloy may be made as a concentrate, e. g., with a high beryllium and silicon content, or beryllium-silicon-copper content, and diluted with aluminium and zinc to form the required alloy. The alloy No. 14 of the foregoing table is one suitable example.

Graphite may be added, e. g., to the zinc-aluminium melt, to promote the sliding properties of the alloy.

The percentages given herein and in the claims hereof are by weight.

What I claim is:

- An alloy consisting essentially of from 20% to 60% aluminium, from 0.15 to 16% silicon, from 0.005% up to 10% of beryllium, and zinc at least 38%.
- An alloy consisting essentially of aluminium at least 20%; silicon from 0.15% to 16%; beryllium from 0.005% to 10%; zinc at least 28%; copper from 0.05% to 6%, iron 0% to 3.5% and not including lead save as an impurity.
- An alloy consisting essentially of from 20% to 75% aluminium, from 0.15% to 16% silicon, from 0.005% up to 10% beryllium, copper from 2.20 to 8% and zinc at least 20%.
- A composition according to claim 1, containing copper per in. the range of .05% to 6%.
- An alloy consisting essentially of 0.50% beryllium, 26.5% aluminium, 0.55% copper, 0.45% silicon, traces of magnesium and the remainder zinc.

References Cited in the file of this patent

UNITED STATES PATENTS

1,879,748 Horsfield Sept. 27, 1932

FOREIGN PATENTS

|    |           |               |               |
|----|-----------|---------------|---------------|
| 25 | 448,929   | Great Britain | June 17, 1936 |
|    | 537,312   | Great Britain | June 17, 1941 |
|    | 638,733   | Great Britain | June 14, 1950 |
|    | 1,001,105 | France        | Feb. 20, 1952 |
|    | 408,097   | Italy         | Dec. 19, 1944 |

OTHER REFERENCES

Jefferies: "Aluminum Industry," pages 307-308, vol. II, McGraw-Hill, New York, N. Y., 1930.